

## UNITED STATES PATENT OFFICE

ROYAL K. ABBOTT, OF CRANSTON, RHODE ISLAND, ASSIGNOR TO RESPRO INC., OF PROVIDENCE, RHODE ISLAND, A CORPORATION OF RHODE ISLAND

## MAKING ARTIFICIAL LEATHER

No Drawing. Application filed April 1, 1937, Serial No. 180,346, and in Great Britain April 7, 1936.

This invention relates to the manufacture of sheet material resembling leather in visual appearance as well as essential physical or structural properties, and employs 5 for its basis sheet materials of the character described in the patent to Roland B. Respass No. 1,524,573 dated January 27, 1925. It is characteristic of that sheet material that at a preparatory stage of its manufacture it consists of a sheet of unwoven fibres, impregnated with a viscid, cementitious substance, but of loose or open texture, which, upon receiving a compressive treatment becomes compact by the integration of previously 10 separate or imperfectly integrated fibre-coatings of the cementitious material. The completed product described in the said patent possesses the structural and physical properties of leather in substantial degree, and is, indeed, stronger than many varieties or 15 grades of leather of equal body thickness. Not only is the stage-product above alluded to permeable by gases—though resistant to penetration by water—but the final compacted product also is like leather permeable by 20 gases, unless the original impregnation by cementitious material be so controlled as to carry into association with the fibres a proportion of the cementitious material so voluminous in its final coagulated, solidified, or 25 dense condition that no interstices remain to permit permeation by gases. This material, when completed by the process described in the said patent, has a dull-appearing 30 surface and therefore requires the application of surface coatings or dressings if it is to simulate finished leather to the eye as well as in its structural and physical properties. Surface coatings or dressings have been applied 35 to such completed material by spreading or dressing machines in the well known manner, substantially as has been the practice in the manufacture of coated cloths, etc. for a long time, and have served their intended purpose 40 satisfactorily except when subjected to conditions which call for great tenacity of union between the material and its coating or dressing if the latter is to remain integrated with the former.

An object of the invention herein described

is to produce a surface-coated or dressed material of the character indicated in which the coating-film is so securely attached to the fibrous material as to be practically inseparable therefrom.

In the practice of this invention, advantage is taken of the structural peculiarities of the stage-product which appears in the manufacture of sheet material in accordance with the process described in the said patent. Instead of coating or surface-dressing the completed material, as heretofore, a loosely constructed sheet of unwoven fibres—such as cotton batting or wadding—is first impregnated with viscid cementitious material—such as 55 rubber or a rubber composition in a solvent vehicle thereof—intruding this into the sheet essentially in the manner described in the said patent; second, the impregnated sheet is allowed, after the first step, to recover part 60 of its original spacial dimension of thickness by virtue of the resiliency of the fibres of which it is composed, so that the impregnated sheet becomes reticular and easily permeable by a fluid (air, in the specific case) 65 which so acts upon the content of viscid cementitious material as to render it much more viscous and adhesively tenacious than it was when intruded into the assemblage of fibres, all substantially as set forth in the said patent. 70

At this stage, the impregnated sheet is relatively soft and loose in texture, though considerably reduced in thickness from its original condition; the constituent fibres are each 75 coated with adhesive cement which is in a condition of augmented tenacity and adhesiveness adapted to bring about and retain a much closer union of the constituent materials upon further compressive treatment. 80 When the material has reached this intermediate stage, before the second or final compressive treatment, there is applied to it and intruded into its pores or cavities from at least one of its surfaces by means of a knife, 85 or other coating instrument, a priming or base coat of dressing. This base coating, according to my application for Letters Patent Serial No. 98,623, filed March 30, 1926 (Patent No. 1,642,394, dated Sept. 13, 1927), may 90

be, for instance, a liquid, viscous or pasty extension or solution of or mixture containing a cellulose derivative, such as nitro cellulose, acetyl cellulose or other cellulose derivative or ester, of such consistency that it interpenetrates the fibrous sheet to the extent of entering the pores of the material and enveloping the fibres (coated with the cementitious material originally introduced) at and near the surface of the material.

This application relates to a surface-coated material of the same generic character as the material of my said application having in addition to or substitution for the cellulosic first coating of said application, a waxy pigment-bearing coating applied in such a way as to increase the adhesive permanence of the surface layer or dressing, and produce a product generically fit for all of the uses of the relatively thin or "upper" leathers, such as for the uppers of shoes, shoe-linings, and miscellaneous leather manufactures such as handbags, purses, book-covers, belts and gloves. This application also relates to a composition of matter suitable for application to the said base material and concatenation with it according to this description.

If the original cementitious impregnant of the fibrous sheet be a rubber composition with gasoline, naphtha, or the like as a solvent vehicle, and the first coating or dressing composition be nitrocellulose extended or dissolved in amyl or ethyl acetate, with or without benzol, or a cellulose acetate extended or dissolved in acetone, the solvent constituent of the dressing remains in wetting contact with, and if benzol or like solvent is used, softens the rubber composition adhering to the surface fibres, in either case forming local association between the soluble constituent of the dressing and the rubber already present, and thus enhancing the intimacy of adhesive association between fibre, rubber and the surface layer and intruded interpenetrating extensions of the dressing material, which now ensues when the sheet material thus supplied with a surface-penetrating base coating or dressing, is subjected to a further compression, as in a calendering or embossing machine. Before finally compressing or calendering the material to its intended state of adhesive integration of fibre-cement inclusion and coating inclusion there may be applied successive coatings of a surface dressing over the base-coat, allowing each coating to set before applying the next; or the application of further surface coatings upon the base coating may be deferred until after the material with the base coating attached has been consolidated by calendering. In either case, each of the successive coatings is preferably of such character as to unite by strong adhesion with the coating to which it is applied. The coatings may be embossed

as well as calendered, to produce whatever superficial appearance is desired. Calendering in some cases may follow embossing for special effects of grain.

When the base coating is applied as above described to the material in its intermediate stage of production and while it is reticular in structure and superficially permeable by a varnish-like coating material, the base coat envelopes the surface fibres, or portions of them, as well as intrudes or penetrates into the grosser cavities of the relatively open unfinished base material, (like the relation of plaster to lathing) so that upon being dried or set to a tacky consistency, the said coating is anchored or tied to the fibres of the sheet material both by adhesion and by intruded keys of the coating. When, at a later stage of manufacture, the coated sheet is heavily compressed, this anchorage or tying of the coating to the fibres, and to the cementitious adhesive material originally applied to the fibres, is rendered so tenacious and secure that the aggregate final finished coating or dressing (composed of several applications of dressing material) is so interlocked with the fibrous body and its cement that any attempt to pull the dressing from the sheet will result in rupture of the latter. This result is effectively produced whether the coating material is cellulosic or waxy, or comprised of layers of each. It will be understood that the first layer or coating having interpenetrated a reticular texture of the fibrous base of which each fibre bears a strongly adhesive coat, the subsequent compression interlocks the coating everywhere within the outer part of the thickness of the base fabric, and conversely that the surface meshes of the reticular base fabric everywhere intrude into the coating, so that on compression the adhesion secured is in part mechanical interlocking and in part adhesive union between the material of base and coating respectively. This relationship applies as well when the open reticular base is subjected to several coatings before compression especially if the first coating does not fill the available interstices, so that when set this coating itself has interstices to be filled by second or later coated layers.

Coating solutions compounded as follows, for an example, yield satisfactory results in application to material having the characteristics above indicated:

For the base coating, nitrated cotton "cut" or dissolved in any of its well-known solvents, e. g. ethyl acetate, to form a 16 oz. solution, so-called (i. e. sixteen ounces of the solute to a gallon of the solvent). To this a pigment ground in castor oil may be added to give a desired color. The addition of castor oil or other softeners may be resorted to in sufficient quantity to produce the desired degree of pliability. When the ingredients used have been thoroughly mixed, the solution is

then thinned by the addition of nitro cellulose solvent until the desired viscosity is obtained. A viscosity of about 28000 centipoises, as given by a Stormer viscosimeter, model 7650-5 A, and calculated by the equations of Higgins & Pitman (Journal of Industrial and Engineering Chemistry, vol. 12,—1920—page 587) is suitable to the purpose.

When a waxy finish of the leather substitute is desirable, the coating applied initially or in succession to the cellulosic coating is recommended to be prepared by the inclusion of a varnish gum and a hard wax in solution with borax and/or soap. The hard wax may be a vegetable or a mineral wax. For example, prepare with stirring a first solution of borax, 17½ pounds; orange shellac flakes, 60 pounds; water, 40 gallons; prepare with heat and stirring a second solution, suspension or extension, of white neutral soap flakes, 6 pounds; carnauba wax, 19 pounds; water, 30 gallons. Mix in the ratio of from five to eight parts of the first solution to three parts of the second solution. The product is a smooth viscid paste, hard but flexible when the water of emulsion or solution has evaporated away, and not water-soluble thereafter to any practical extent. This dressing paste contacts without resistance to adhesion with the viscid rubber cement of the base fabric. Pigments may be ground in the second solution, and sufficient quantities of perfumes, such as the oils of sassafras, citronella, birch, origanum oil may be mixed with either solution to impart a desirable odor. This dressing may be spread on and intruded into the open pores of the fabric, with or without a first coating of colloidal material as above described, dried, and thereafter subjected to the described compacting pressure.

The varnish gum for the first solution is preferably a shellac which has not been subjected to solution in any alcoholic, etheric or ketonic solvent.

Before or after the application of a coating of this waxy dressing, and after or during the heavy compressive integration of the fabric by pressure necessary to the completion of the fibre-and-cement base fabric, the material may be subjected to embossing in imitation of any of the natural or artificial leather grains, or with any arbitrary pattern. When the dressing is set and dry, the surface may be subjected to any desirable treatment. For example, a liquid or powdered pigmenting coat in a contrasting color may be applied, and with or without this, the surface may be finished or polished by brushing or buffing, or both.

The coated sheet, made as above described, has been found entirely adequate in many respects to the manufacture of shoes, novelties, pocket-books, trunk linings, book covers and book bindings as a substitute for leather.

The flections and creasings to which the ma-

terial described is subjected when used as parts or as a whole of the leather-like parts of such articles have no effect on the coating, which remains tenaciously attached to the tough fibrous sheet material. 70

I claim:

1. Composition of matter adapted for coating an artificial leather of the kind having a cement-integrated unwoven fibrous base by application in the open reticular state of said base comprising a varnish gum, in solution, and a hard wax and a neutral soap dispersed in an aqueous menstruum. 75
2. Composition of matter adapted for coating artificial leathers comprising a varnish gum and a wax respectively held in aqueous solution by a saponifying agent, and in dispersion by a soap, and mixed. 80
3. Composition of matter adapted for coating artificial leathers comprising shellac and a hard vegetable wax respectively held in aqueous solution by a saponifying agent, and in dispersion in said solution. 85
4. Composition of matter adapted for coating artificial leathers comprising a varnish gum and a wax respectively held in aqueous solution and in suspension by saponifying agents, and a suitable pigment dispersed therein. 90
5. Composition of matter adapted for coating artificial leathers comprising a varnish gum and a wax respectively held in aqueous solution and in suspension by saponifying agents, and an odorous vegetable oil. 95
6. Composition of matter comprising a mixture of suitable proportions of first an aqueous solution of shellac in water with the aid of borax, and second of carnauba wax dispersed in water with the aid of soap, one of said aqueous solutions carrying a suitable pigment dispersed therein in finely-divided homogeneous distribution. 100
7. Composition of matter comprising a mixture of a quantity of an aqueous solution of shellac in water with the aid of borax and of a lesser quantity of carnauba wax dispersed in water with the aid of soap, one of said aqueous solutions carrying a suitable pigment dispersed therein in finely-divided homogeneous distribution. 110
8. Composition of matter comprising a mixture of suitable proportions of first an aqueous solution of shellac in water with the aid of borax, and second of carnauba wax dispersed in water with the aid of soap, one of said aqueous solutions carrying a suitable pigment dispersed in finely-divided homogeneous distribution therein, and one of said solutions having dispersed therein a suitable quantity of an odorous vegetable oil. 120

Signed by me at Providence, Rhode Island, this 30th day of March, 1927.

ROYAL K. ABBOTT.